

# UNITED STATES PATENT OFFICE.

JULIEN VERMEESCH, OF SCHAERBEEK, BELGIUM.

## METHOD OF MANUFACTURING TEXTILE FIBERS OR ARTIFICIAL SILK.

No. 836,620.

Specification of Letters Patent.

Patented Nov. 20, 1906.

Application filed April 9, 1906. Serial No. 310,857.

*To all whom it may concern:*

Be it known that I, JULIEN VERMEESCH, a subject of the King of Belgium, residing at Schaerbeek, Belgium, have invented a certain new and useful Method of Manufacturing Textile Fibers or Artificial Silk, of which the following is a specification.

This invention relates to an improved method of manufacturing brilliant or glossy textile fibers by means of solution of cellulose in copper-ammonia.

The invention relates to that kind of manufacture of brilliant fibers in which the material is discharged through capillary orifices and passes under pressure into a precipitating-bath, from which it is removed in order to be wound on spools, &c.

The object of the invention is to obtain specially supple, brilliant or glossy, and very strong filaments.

It also has for its object to decrease in the artificial-silk industry the elements injuriously affecting the health of the workmen and the durability of the machinery, and finally to allow a great portion of the chemical agents used for the manufacture and precipitation of filaments to be recovered for reuse.

The invention chiefly consists in introducing jets of solution of cellulose escaping from capillary orifices into a precipitating-bath consisting of acidulated or alkalized glycerin.

Owing to the combined and simultaneous action of the glycerin and of the acid or of the glycerin and of the alkali, an energetic and quick precipitation is obtained, acting at once on the whole section of the filament and enabling textile fibers to be obtained which while being very strong and water-resistant have an exceedingly brilliant or glossy appearance. The fibers are translucent and exceedingly silky, surpassing anything it has been possible to obtain up to now. On being discharged from the precipitating-bath the threads are introduced into a washing-bath and for that purpose are wound on glass spools immersed in a solution of glycerin and water, which dissolves the copper salts and decolorizes the filaments. A rinsing in clear water, followed by drying, completes the process of manufacture.

In order to obtain a specially energetic and quick action of the precipitating liquid and at the same time to increase its mercerizing action, the precipitating agent is preferably

prepared in a special manner, which will be now described. To two parts of sulfuric acid (density 1.84) is slowly added one part of pure glycerin. It is important to make this mixture very slowly, so as to avoid strong generation of heat, which would transform the glycerin partly into acrolein and produce secondary products disengaging acrid fumes, blackening the liquid, and rendering it unsuitable for use as a precipitating-bath. The result of this operation is the production of glycerylmonosulfuric acid,  $C_3H_5(OH)_2SO_4H$ . (See Würtz, first part, page 1589.) The liquid is cooled by means of any suitable device, and an equal volume of water is added to it. Then the cooling is continued and another quarter part of glycerin is added. The liquid in question is therefore constituted by thirty-seven and one-half per cent. of glycerylmonosulfuric acid, thirty-seven and one-half per cent. of water, and twenty-five per cent. of glycerin, and this liquid forms the precipitating-bath, into which is introduced the solution of cellulose discharged under a strong pressure (one and one-half to two atmospheres) in the shape of threads from capillary tubes with an exceedingly small section of passage, (the diameter of the discharge-orifice being as low as 0.15 or even 0.12 of a millimeter.)

The precipitating action of the solution of glycerylmonosulfuric acid on the solution of cellulose is very energetic and quick, while the presence of the last addition of glycerin (not combined and simply in solution) is a special and useful feature. It increases, in fact, the mercerizing action of the bath, renders the thread more supple, and prevents the threads from sticking to each other on the winding-spool, and, moreover, its dissolving action on the non-reduced oxid of copper is obvious. In view of the rapidity of the precipitating action of the mixture on the solution of cellulose in very thin threads it is advisable, in order to obtain all the desirable results, to remove it from the thread as quickly as possible. To that end it is necessary, first of all, to reduce to the strict minimum required the duration of the contact of the threads with the precipitating liquid. To that effect the capillary orifices are preferably arranged relatively to the precipitating liquid in such manner that the discharge-orifices are at a small distance below the level of the liquid in a tank of such capacity as it will not become saturated too quickly. Ex-

perience has shown that by arranging the capillary tubes so that they are immersed to the height of about two centimeters the duration of the passage of the filaments through 5 the precipitating liquid is regulated in the most advantageous manner; but at the same time the speed of winding of the thread must not be too great. The thread is wound on a spool arranged outside the bath at a speed of 10 seventy-five to one hundred revolutions per minute. Secondly, it is necessary to stop immediately on leaving the bath the action of the glycerylmonosulfuric acid carried away by the thread, which is effected by treating 15 the thread with a neutralizing liquid consisting, say, of a solution of chlorid of sodium in water. The glycerin carried away by the threads and that released actuate the solution of the non-reduced oxid of copper and 20 continue to act on the thread in order to give it perfect suppleness. Other salts than chlorid of sodium could be used for the same purpose. Such, for instance, are, generally speaking, all soluble salts of organic acids 25 and minerals in which sulfuric acid can be substituted for the constituent acid—formate, acetate, oxalate, alkaline chlorids, chlorids of alkaline earth, &c. If on leaving the chlorid-of-sodium bath the spool is not completely 30 decolorized, it is submitted to washing in a very dilute solution of bisulfate of soda, which immediately fixes the remaining copper. Then the spool is washed in pure water.

What I claim as my invention, and desire 35 to secure by Letters Patent, is—

1. A method of manufacturing glossy textile fibers from a solution of cellulose in copper-ammonia, discharged in the shape of fine jets from capillary orifices consisting in causing 40 the threads to pass through a precipitating liquid constituted by a solution of glycerylmonosulfuric acid in water mixed with glycerin, and subsequently introducing them into a neutralizing-bath consisting of a soluble salt in which sulfuric acid can be substituted for the constituent acid, dissolving the 45 copper salts left in the filaments, precipitated by the glycerin, in a solution of bisulfate of soda in water, and finally washing in pure water containing, if desired, a small quantity of glycerin, as set forth.

2. A method of manufacturing glossy textile fibers from a solution of cellulose in copper-ammonia discharged in the shape of fine jets from capillary orifices consisting in causing 50 the threads to pass through a precipitating liquid constituted by a solution of glycerylmonosulfuric acid in water mixed with glycerin, and subsequently introducing them 55 into a neutralizing-bath consisting of a solution of sodium chlorid in water, substantially as set forth.

3. A method of manufacturing glossy textile fibers from a solution of cellulose in copper-ammonia, discharged in the shape of fine jets from capillary orifices consisting in causing 60 the threads to pass through a precipitating liquid constituted by a solution of glycerylmonosulfuric acid in water mixed with 65 glycerin, and subsequently introducing them into a neutralizing-bath consisting of a soluble salt in which sulfuric acid can be substituted for the constituent acid, and washing the threads in a diluted solution of bisulfate 70 of soda, substantially as set forth.

4. A method of manufacturing glossy textile fibers from a solution of cellulose in copper-ammonia, discharged in the shape of fine jets from capillary orifices consisting in causing 75 the threads to pass through a precipitating liquid constituted by a solution of glycerylmonosulfuric acid in water mixed with glycerin, and subsequently introducing them into a neutralizing-bath consisting of a soluble salt in which sulfuric acid can be substituted for the constituent acid, dissolving the 80 copper salts left in the filaments, precipitated by the glycerin, in a solution of bisulfate of soda in water, and finally washing in pure 85 water containing, if desired, a small quantity of glycerin, as set forth.

In testimony whereof I have signed my name to this specification in the presence of two subscribing witnesses.

JULIEN VERMEESCH.

Witnesses:

A. GRAETZ,  
GREGORY PHELAN.